

April 30, 1968

TADAO SENOO ET AL

3,381,057

CRIMPED POLYESTER FILAMENTS

Filed May 2, 1966

FIG. 1



FIG. 2



INVENTORS  
Tadao Senoo  
Yoshiro Ono  
Pierre Grentz  
Attorney  
BY

1

3,381,057

### CRIMPED POLYESTER FILAMENTS

Tadao Senoo and Yoshizo Onaya, Asaka-gun, Fukushima-ken, Japan, assignors to Nitto Boseki Company Limited, Fukushima-ken, Japan, a corporation of Japan

Filed May 2, 1966, Ser. No. 546,887

6 Claims. (Cl. 260—860)

### ABSTRACT OF THE DISCLOSURE

A polyester filament composition which comprises 50–100 parts by weight of a highly crystalline and rapid crystallizing homopolyester selected from the group consisting of a homopolyester obtained from polymerizing 1,2-bis-(carbomethoxyphenoxy)-ethane with ethylene glycol and homopolyester being polyethylene terephthalate, and said homopolyester being blended with 40–100 parts by weight of a block copolymer resulting from the polymerization of said homopolyester with a polyethylene glycol having a molecular weight of 1,000–6,000.

The present invention relates to the manufacture of crimped polyester filaments and has particular reference to the process for producing highly crimped filaments or fibers by spinning homopolymers together with block copolymers of said homopolymers and polyethylene glycol.

There has been introduced a number of processes for the production of various synthetic fibers by spinning different types of polymers in a molten state.

One of the drawbacks inherent in such prior-art processes is that the filaments thereby obtained are difficult to be crimped for the reason that the filament components are cross-sectionally homogeneous and symmetric in the chemical or physical properties.

This drawback has been overcome in one way by mechanically forcing the filaments to be crimped with use of, for example, a toothed gear-wheel.

Such mechanical means, however, would provide only two-dimensional crimps in the filaments which tend to get released with time. Another way of providing crimps in the filaments heretofore proposed is based on the discovery that heterogeneity and asymmetry of the physico-chemical properties of starting polymers are conducive to the crimping effect, as this is exemplified by acryl filaments trade named "Orlon 21." Examination of the cross section of this acryl fiber shows that it comprises two distinctive regions—hydrophilic and hydrophobic—which add to easiness of crimping.

More lately known for the preparation of highly crimped artificial filaments is a so-called "conjugate-spinning" wherein two or more different types of polymers are separately melted or dissolved and spun through the respective nozzles, immediately followed by combining all individual streams of polymers into a single piece of filament. This process is extremely complicated from the practical, commercial point of view and further has the disadvantage that the filaments after spun are often apt to disintegrate back into individual components.

Whereas, it is an object of the present invention to provide improved method and means for producing highly crimped filaments of this character which will eliminate the above-noted difficulties.

It is another object of the present invention to provide highly crimped artificial filaments of this character which have excellent fastness to light, color, wash and sublimation, good affinity to dye and other requisite properties for fibers and fabrics.

These and other advantages and features of the present invention will be more apparent from the detailed de-

2

scription which follows in conjunction with a few preferred embodiments of the inventive concept, a reference being had to the accompanying drawings wherein:

FIG. 1 is a schematic illustration revealing the cross-sectional features of the filament of the present invention as observed under a microscope, and

FIG. 2 graphically displays the residual tenacity and elongation factors of the filament of the present invention as plotted against time of light exposure irradiation.

10 The present inventors have discovered that polyester filaments of such desired properties as set forth in the above objects of the invention may be obtained by blending two or more polymeric materials which are cosoluble but significantly differ from each other in the crystallinity and velocity of crystallization.

It has been further discovered that some components of such polymer mixture melt and mingle uniformly with other components but tend to crystallize faster than the latter when extruded through a nozzle. This is because the 20 former component polymers have remarkably higher crystallinity and faster crystallization tendency than the latter. The use of two or more of these characteristically different polymers gives intensive crimps to the resulting filaments, the form of such crimps being substantially 25 helical according to the present invention.

The higher crystallinity and faster crystallization type of polymer according to the invention may preferably be polyethylene terephthalate or a polyester resulting from the reaction of 1,2-bis-(carbomethoxyphenoxy)-ethane 30 with ethylene glycol. Whereas, the lower crystallinity and slower crystallization category of polymer may preferably be a block copolymer resulting from the polycondensation of dimethyl terephthalate and ethylene glycol to form polyethylene terephthalate in the presence of 35 polyethylene glycol. The structural formula of this block copolymer is:



40 where  $m$  and  $n$  represent polymerization degrees, and this 45 polymer contains 10%–60% by weight of the polyethylene glycol component (2).

Another example of block copolymer according to the 50 invention may be obtained from the polycondensation of 1,2-bis-(carbomethoxyphenoxy)-ethane and ethylene glycol to form a polyester in the presence of polyethylene glycol. This is represented by the structural formula:



55 where  $m$  and  $n$  represent polymerization degrees, and this 60 polymer contains 10%–70% by weight of the polyethylene glycol component (4).

Molecular weight of the polyethylene glycol used in the formation of each block copolymer may preferably 65 be in the range of 1,000 to 6,000.

Experiments revealed that excellent results may be obtained particularly with the above two block copolymers when admixed at predetermined ratios respectively with polyethylene terephthalate and a polyester resulting from the polymerization of 1,2-bis(carbomethoxyphenoxy)-ethane and ethylene glycol. Preferred amounts of the block copolymer (I) to be admixed with polyethylene



substantially helical form, the number of crimp waves increasing to about 10 to 20.

Example 4

A white block copolymer was used which was the same as used in Example 1 except that 70 parts by weight of dimethyl terephthalate were polymerized with 30 parts of polyethylene glycol. This block copolymer having a specific viscosity of 1.650 and a melting point of 240°-243° C. was pelletized to a size measuring 2 mm. in diameter and 3 mm. long.

50 parts by weight of these pellets were admixed with 50 parts of polyethylene terephthalate pellets and spun in the manner described in Example 3. The resulting filament, when stretched by four times, revealed 5 to 10 helical crimp waves per 10 mm. length. It was further heated to 100° C. for about 10 minutes thereby increasing the number of crimp waves to about 15 to 20. The thus thermally set filament was tested to show a fineness of 5.32 deniers, a tenacity of 3.37 grams per denier, an elongation of 44.5%, an average number of crimp waves amounting to 15.8 per 10 mm. length and a crimp elasticity of 73.4%.

Since the invention has been described in some detail as to a few specific embodiments thereof, it will be understood that certain changes and adaptations may be made as obvious to those skilled in the art without departing from the accepted claims in which it is the intention to claim all novelty inherent in the invention as broadly as is permissible in view of the prior art.

What is claimed is:

1. A polyester filament composition comprising 50-100 parts by weight of a highly crystalline and fast crystallizing homopolyester, selected from the group consisting of polyethylene terephthalate and the polyester obtained by polymerizing 1,2-bis-(carbomethoxyphenoxy)-ethane with ethylene glycol, blended with 40-100 parts by weight of a block copolymer resulting from the polymerization of said homopolyester with a polyethylene glycol having a molecular weight of 1,000-6,000.

2. A polyester filament as defined in claim 1, wherein said homopolyester is obtained from polymerizing 1,2-bis-(carbomethoxyphenoxy)-ethane with ethylene glycol.

3. A polyester filament as defined in claim 1, wherein said homopolyester is polyethylene terephthalate.

4. A process for the production of highly crimped polyester filaments comprising pelletizing 100 parts by weight

of a block copolymer resulting from the polymerization of 1,2-bis-(carbomethoxyphenoxy)-ethane, ethylene glycol and polyethylene glycol having a molecular weight of 1,500-3,000, admixing said block copolymer with 100 parts of similarly pelletized homopolyester resulting from the polymerization of 1,2-bis-(carbomethoxyphenoxy)-ethane and ethylene glycol heating the admixture to 260°-280° C. and melt spinning thereby producing sharply crimped filaments and thermally setting said filaments at 100° C.

5. A process for the production of highly crimped polyester filaments comprising pelletizing 40 parts by weight of a block copolymer having a specific viscosity of 1.653 and a melting point of 226°-230° C. resulting from the polymerization of 1,2-bis-(carbomethoxyphenoxy)-ethane, ethylene glycol and polyethylene glycol having a molecular weight of 1,500-3,000, admixing same with 60 parts of similarly pelletized homopolyester resulting from the polymerization of 1,2-bis-(carbomethoxyphenoxy)-ethane and ethylene glycol, heating the admixture to 260°-280° C. for melt spinning thereby producing sharply crimped filaments and thermally setting said filaments at 100° C. for about 10 minutes.

6. A process for the production of highly crimped polyester filaments comprising pelletizing 40-50 parts by weight of a block copolymer having a specific viscosity of 1.650-1.831 and a melting point of 238°-243° C. resulting from the polymerization of dimethyl terephthalate, ethylene glycol and polyethylene glycol having a molecular weight of 1,500-3,000, admixing same with 40-60 parts of similarly pelletized polyethylene terephthalate, heating the admixture to 260°-280° C. for melt spinning thereby producing sharply crimped filaments and thermally setting said filaments at 100° C.

References Cited

UNITED STATES PATENTS

|           |           |                       |         |
|-----------|-----------|-----------------------|---------|
| 2,836,576 | 5/1958    | Piccard et al. -----  | 260-860 |
| 40        | 3,013,914 | 12/1961 Willard ----- | 164-43  |

FOREIGN PATENTS

|         |        |                |
|---------|--------|----------------|
| 777,574 | 6/1957 | Great Britain. |
| 956,833 | 4/1964 | Great Britain. |

45 MURRAY TILLMAN, Primary Examiner.

JOHN T. GOOLKASIAN, Assistant Examiner.